

Jan. 14, 1964

**E. GORIN**

3,117,921

## PRODUCTION OF HYDROGEN-ENRICHED LIQUID FUELS FROM COAL

Filed Jan. 21, 1963



1

3,117,921

PRODUCTION OF HYDROGEN-ENRICHED  
LIQUID FUELS FROM COALEverett Gorin, Pittsburgh, Pa., assignor to Consolidation  
Coal Company, Pittsburgh, Pa., a corporation of  
Pennsylvania

Filed Jan. 21, 1963, Ser. No. 252,822

5 Claims. (Cl. 208—8)

The present invention relates to a process for the production of hydrogen-enriched liquid fuels from coal.

This application is a continuation-in-part of my copending application Serial No. 144,428, filed October 11, 1961, now abandoned, which is assigned to the assignee of the present application.

Hydrogen-enriched liquid fuels such as gasoline, diesel oils, fuel oils, kerosene, and the like represent more than one-third of the total annual United States' natural energy production, and from all indications, the demand for such liquid fuels will increase in the years to come. At the present time the principal source of such liquid fuels is petroleum; however, for many years researchers have been attempting to design economic processes of commercial utility for producing such liquid fuels from solid materials such as coal.

One approach to the production of synthetic hydrogen-enriched liquid fuels from coal involves coal solvent extraction wherein the coal is extracted to yield coal extract which thereafter is hydrogenated to yield the desired liquid fuels. Heretofore, all of the resulting extract was completely converted via hydrogenation to the desired fuels in one or more stages at elevated temperatures and pressures in the presence of a catalyst. I have now found that coal extract varies in its reactivity to hydrogenation and consequently it is desirable, economically, to convert via hydrogenation only a portion of the coal extract to the desired liquid fuels. For example, at a given set of hydrogenation conditions a portion of the extract will be converted to the desired liquid fuels. In order to convert the remaining unconverted extract to the same liquid fuels, more severe hydrogenation conditions are required, which in most instances substantially increase the cost of the over-all coal conversion process.

The primary object of the present invention is to provide an improved process for producing hydrogen-enriched liquid fuels such as gasoline from coal.

In accordance with my invention, coal is subjected to solvent extraction under conditions to dissolve up to 80 weight percent of the coal (on a moisture-free and ash-free basis). The coal extraction product, which comprises coal extract and undissolved coal residue, is then treated, for example, in a filtration zone, to separately recover coal extract. This extract, which is a solid at room temperature and which is substantially free of hydrocarbons boiling below 400° C., is composed almost entirely of nondistillable, high molecular weight polycyclic aromatics. These polycyclic aromatics differ substantially in their response to hydrogenation treatment at elevated temperatures. I have observed that if the hydrogenation conditions are dictated by the more refractory components of the extract, then an inordinate amount of coke and gas is produced. Accordingly, in my improved process the extract is subjected to a prehydrogenation treatment which effects only partial conversion of the extract to a distillable liquid boiling below 325° C. In general, the prehydrogenation is conducted at a temperature between 400 and 470° C. and at a pressure between 500 and 5,000 p.s.i.g. However, the conditions may fall somewhat outside these ranges depending on the nature of the extract or on the selection of catalyst, if any. A higher boiling or so-called bottoms portion of the prehydrogenated extract is subjected to carbonization, i.e. coking, at 425 to 760° C., to

2

yield a liquid distillate. A lower boiling portion of the prehydrogenated extract in admixture with at least a portion of the liquid distillate is subsequently hydrogenated to yield hydrogen-enriched liquid fuels.

For a better and more complete understanding of my invention, its objects and advantages, reference should be had to the following description and to the sole FIGURE of the accompanying drawing which is an illustration of the preferred embodiment of the present invention.

## Preferred Embodiment

Referring to the drawing, coal, preferably high volatile bituminous coal, is introduced into a stirred solvent extraction zone 10 concurrently with 0.5 to 4.0 parts by weight of a coal extraction solvent. The extraction zone 10 is adapted to confine the coal and the solvent for a residence period from about five minutes to four hours at elevated pressures and temperatures. The residence period and temperatures are determined by the specific solvent and the desired depth of coal extraction. The pressure is preferably that required to maintain the solvent as a liquid at the selected temperature, generally in the range of 1 to 6500 p.s.i.g.

Suitable solvents for the coal in the extraction step are those which are predominantly polycyclic, aromatic hydrocarbons, preferably partially or completely hydrogenated aromatics, including completely saturated naphthenic hydrocarbons which are liquid under the temperature and pressure of extraction. Mixtures of these hydrocarbons may be used and are preferably derived from intermediate or final steps of the process of this invention. Those hydrocarbons or mixtures thereof boiling between about 260 and 425° C. are especially preferred. Examples of suitable solvents are tetrahydronaphthalene, decalin, biphenyl, methylnaphthalene, and dimethylnaphthalene. Other types of coal solvent may be added to the above-mentioned types for special reasons, but the resulting mixture should be predominantly of the types mentioned. Examples of additive solvents are the phenolic compounds such as phenol, cresols, and xylenols.

The coal and the solvent are maintained in intimate contact within the extraction zone 10 until the solvent has dissolved, i.e., converted the desired amount of coal. Preferably up to 80 weight percent of the MAF (MAF signifies moisture-free and ash-free) coal is dissolved, as is further discussed in my U.S. Patent No. 3,018,241. It has been found that the cost of converting more than 80 weight percent of the coal becomes economically prohibitive in terms of the amount of hydrogen transfer that is needed. In addition, as the depth of coal extraction is increased, each additional increment of coal extract contains a higher proportion of benzene-insoluble material which correspondingly makes the resulting coal extract more difficult to hydrogenate. If desired, however, any depth of coal conversion may be used. In fact, if more than 80 weight percent coal conversion is used, the process of the present invention becomes even more desirable. I have found that it is particularly preferred to conduct the solvent extract under conditions to yield an extract amounting to less than 60 weight percent of the MAF coal.

The temperature of the extraction zone should be an elevated temperature between about 100 and 500° C., but preferably not high enough to cause appreciable coke formation. In some instances it may be desirable to conduct the coal extraction in stages at successively higher temperatures until the desired depth of extraction is attained. Instead of a batch system, a continuous or a countercurrent system may be employed. The particular system used is not material to the practice of my invention.

Following extraction, the mixture of solvent, extract,

and residue is conveyed through a conduit 12 to a conventional type separation zone 14 such as a filtration zone, sedimentation zone, or centrifugation zone. The extract, which is usually a solid at room temperature and generally contains less than 5 weight percent hydrocarbons boiling below 400° C., is therein separated from the residue. If desired, a portion of the coal extract may be separated with the residue and processed therewith. For example, in my U.S. Patent No. 3,018,241, it is shown that the extract may be cooled or treated with a paraffinic solvent such as hexane to separate the extract into a benzene-soluble rich extract fraction and a benzene-insoluble rich extract fraction. The latter extract fraction may be coked alone or in combination with the residue.

The residue, alone or in combination with a precipitated benzene-insoluble rich extract fraction, is conveyed via a conduit 16 to a drying zone 18 wherein a recycle gas stream entering through a conduit 20 is used to strip any retained solvent therefrom. The effluent stream from the drying zone 18 is passed through a conduit 22 to a pair of cyclone separators 24 and 25 which separate the vapors from the solids. The solids drop into a conduit 26 where they are picked up by a carrier gas and introduced into a carbonization zone 28.

The carbonization zone 28 may be any one of the well-known systems for carbonizing carbonaceous solids at low temperatures, i.e. 425 to 760° C. For example, solids may be maintained in the zone in a fluidized bed by means of the above-mentioned carrier gas. The temperature of the carbonization zone may be maintained by any suitable means, for example, by preheating the carrier gas to the appropriate high temperature or by burning a portion of the carbonized residue, i.e., char, produced in the carbonization zone 28. This latter method is accomplished by withdrawing char from the carbonization zone 28 through a conduit 30, and conveying the withdrawn char by means of an inert gas such as recycle gas entering through a conduit 32, into a char devolatilization zone 34. The char is preferably maintained in a fluidized bed in the zone 34 at a temperature between about 645 and 945° C. The devolatilization temperature must be higher than any processing temperature to which the solids have been previously exposed. The volatile content of the solids will be driven off as a hydrogen-rich gas which can be recovered through a conduit 36.

A portion of the devolatilized char is withdrawn from the devolatilization zone 34 through a conduit 38, picked up by air entering through a conduit 40, and lifted through a combustion leg 42. The temperature of the char as a result of the combustion is raised to that sufficient to maintain the temperature in the devolatilization zone 34 when returned through a cyclone separator 44 and a conduit 46 to that zone. Flue gas is removed from the cyclone separator 44 through a conduit 48. Hot char from the devolatilization zone 34 is transferred by a conduit 50 back to the carbonization zone 28 by means of recycle gas from the conduit 32. Net char produced in the carbonization zone 28 is discharged through a conduit 52.

The hydrogen-rich gas from the char devolatilization zone 34 is conducted via the conduit 36 to a conversion zone 54 wherein substantially pure hydrogen is produced by techniques well known in the art, as is further explained in my copending application Serial No. 144,423, filed October 11, 1961, and assigned to the assignee of this invention. The resulting hydrogen may be used, for example, in the subsequent hydrogenation of the extract.

Returning to the carbonization zone 28, the effluent tar vapors are circulated through cyclone separators 56 and 58, which return finely divided solids to the carbonization zone 28. The distillate tar vapors are withdrawn from the carbonization zone via a conduit 60 and subsequently fractionated, as more fully explained hereinafter.

Returning now to the coal extract which is separated from the residue in the separation zone 14, the extract

is conducted through a conduit 62 to a flash tower 64 wherein at least some of the solvent is flashed off through a conduit 66. The solvent vapors are commingled with solvent vapors from the afore-mentioned residue drying zone 18 in a conduit 68 which carries the solvent vapors to a condenser 70. Any noncondensable gas is discharged through a conduit 72 while the condensed solvent is returned to the extraction zone 10 via a conduit 74.

The extract is conveyed from the flash tower 64 through a conduit 76 to a preheater 78 which serves to raise the temperature of the extract to about 426 to 468° C. The preheated extract is passed through a mild prehydrogenation zone 80 which serves to add about 0.5 to 2.0 pounds of hydrogen per 100 pounds of feed. The operating conditions are as follows:

Temperature ----- 425 to 470° C.  
Pressure ----- 500 to 2500 p.s.i.g.  
Residence time ---- 5 to 60 minutes, preferred 10 to 30 minutes.

Hydrogen input to the prehydrogenator 80 may be by means of hydrogen transfer from hydrogenated oil derived from a final step of the present process. Free hydrogen gas may also be added to aid hydrogenation. The prehydrogenation operation is preferably conducted substantially noncatalytically, or with relatively small amounts of "homogeneous" catalysts, i.e., 0.05 to 1.0 weight percent of a hydrogen halide or its corresponding ammonium salt, i.e., NH<sub>4</sub>Cl, NH<sub>4</sub>Br, or NH<sub>4</sub>I. Inexpensive catalysts such as red mud may also be used if desired. The hydrogenated oil is used in amounts between 1 and 3 parts per part of extract, preferably mixed with solvent from the flash tower 64.

The mildly prehydrogenated extract is discharged through a conduit 82 into a fractionation zone 84 which preferably separates the prehydrogenated extract products into a +325° C. and a -325° C. fraction. The latter fraction is withdrawn through a conduit 85 and subsequently hydrogenated. The +325° C. bottoms fraction which still contains nondistillable hydrocarbons is conveyed through a conduit 86 into a conduit 88 to a preheater 90, and thence through a conduit 92 to a coking zone 94 operating at 425 to 760° C. Ash-free coke is discharged through a conduit 96. Coker distillate is withdrawn from the coking zone 94 via a conduit 98 and is commingled with the distillate tar vapors withdrawn from the carbonizer 28 via a conduit 60. The distillate mixture is introduced into a fractionation zone 100. A -300° C. fraction is recovered through a conduit 102 for further refining, if desired, to yield chemicals and low boiling solvents. A 300 to 425° C. fraction is sent through a conduit 104 to a preheater 105. The preheated fraction is withdrawn via a conduit 106 and thence admixed in the conduit 85 with the -325° C. fraction of the prehydrogenated extract. The mixture is then introduced into a hydrogenation zone 110. The portion of the distillates boiling above 425° C. is withdrawn from the fractionation zone 100 via a conduit 109 and recycled to the coking zone 94.

In the hydrogenation zone 110, the prehydrogenated extract and tar are contacted with hydrogen, preferably in the presence of a hydrogenation catalyst. Hydrogenation of the extract and tar may be conducted at pressures of 1000 to 10,000 p.s.i.g., preferably about 2000 to 3500 p.s.i.g., a range well below that normally required for direct hydrogenation of coal. The hydrogenation temperature range is about 400 to 600° C., preferably about 410 to 455° C. The hydrogenation catalyst should be sulfur-resistant, e.g., molybdenum or tungsten oxides or sulfides impregnated on a refractory support to permit catalyst regeneration. The support usually will be an alumina-rich material such as pure gamma alumina or alumina composited with other oxides such as silica. Other metals such as nickel or cobalt may be added as catalyst promoters.

The products of hydrogenation are discharged from the hydrogenation zone 110 through a conduit 112, cooled, and passed into a fractionation zone 114 wherein the products are separated into any desired fractions. A preferred separation is to fractionate the hydrogenation product into a fraction boiling above 360° C. and a fraction boiling below 360° C. The latter fraction is passed through a conduit 116 to further refining and hydrogenation operations for conversion to gasoline. The former fraction is passed through a conduit 118 and may be reintroduced into the hydrogenation zone 110 or into the coking zone 94. If desired, portions of both fractions may be introduced into the solvent extraction zone 10 as a part of the solvent therein.

According to the provisions of the patent statutes, I have explained the principle, preferred construction, and mode of operation of my invention and have illustrated and described what I now consider to represent its best embodiment. However, I desire to have it understood that, within the scope of the appended claims, the invention may be practiced otherwise than as specifically illustrated and described.

I claim:

1. A combination process for the production of hydrogen-enriched liquid fuels from coal, which comprises
  - (a) subjecting the coal to solvent extraction to yield a mixture of extract and undissolved coal residue,
  - (b) recovering from said mixture at least a portion of said extract which is substantially free of hydrocarbons boiling below 400° C.,
  - (c) subjecting said extract portion to prehydrogenation to effect only partial conversion thereof to a distillable fraction boiling below 325° C.,
  - (d) subjecting at least a portion of the +325° C. product from step (c) to carbonization to yield a liquid distillate,
  - (e) combining at least a portion of said liquid distillate of carbonization and a lower boiling portion of the product from step (c), and
  - (f) thereafter hydrogenating the resulting mixture to yield hydrogen-enriched liquid fuels.
2. A combination process for the production of hydrogen-enriched liquid fuels from coal, which comprises
  - (a) subjecting the coal to solvent extraction to yield a mixture of extract and undissolved coal residue,
  - (b) separating at least a portion of said extract from said residue,
  - (c) subjecting the extract to mild prehydrogenation at

5

a temperature between 425 and 470° C. and at a pressure between 500 and 2500 p.s.i.g. to yield prehydrogenated extract,

- (d) subjecting a higher boiling fraction of said prehydrogenated extract products to carbonization at 425 to 760° C. to yield a liquid distillate,
- (e) combining at least a portion of said liquid distillate of carbonization and a lower boiling fraction of said prehydrogenated extract products, and
- (f) thereafter hydrogenating the resulting mixture to yield said hydrogen-enriched liquid fuels.

3. The process of claim 2 wherein said undissolved coal residue is subjected to carbonization in a fluidized low temperature carbonization zone at a temperature between 425 and 760° C. to yield a liquid distillate, at least a portion of which is subjected to hydrogenation in step (f).

4. The process of claim 2 wherein said coal is subjected to solvent extraction under conditions to dissolve less than 80 weight percent of the moisture-free and ash-free coal, whereby a mixture of extract and undissolved coal residue is obtained.

5. A combination process for the production of hydrogen-enriched liquid fuels from coal which comprises

- (a) subjecting the coal to solvent extraction under conditions to yield an extract amounting to less than 60 percent by weight of the moisture-free and ash-free coal and containing both benzene-soluble and benzene-insoluble material,
- (b) separating the extract from the undissolved coal residue,
- (c) subjecting said residue to carbonization under conditions yielding a liquid distillate,
- (d) subjecting the extract to mild prehydrogenation under substantially noncatalytic conditions at 425 to 470° C. and 500 to 2500 p.s.i.g. until about 0.5 to 2.0 pounds of hydrogen per 100 pounds of extract have been added to said extract,
- (e) subjecting at least a higher boiling portion of said prehydrogenated extract to carbonization at 425 to 760° C. to yield a liquid distillate,
- (f) combining said liquid distillates of carbonization,
- (g) subjecting the resulting mixture to hydrogenation under catalytic conditions at 400 to 600° C. and 1000 to 10,000 p.s.i.g., and
- (h) recovering the hydrogenated products.

No references cited.